

# United States Patent

Heuschkel

[15] 3,635,698

[45] Jan. 18, 1972

[54] **HIGH-STRENGTH, HIGH-TOUGHNESS  
(IRON-CARBON-NICKEL-  
MOLYBDENUM) STEEL WELD METAL**

[72] Inventor: Julius Heuschkel, Irwin, Pa.

[73] Assignee: Westinghouse Electric Corporation, Pittsburgh, Pa.

[22] Filed: Apr. 7, 1970

[21] Appl. No.: 26,230

[52] U.S. Cl..... 75/123 J, 75/123 K

[51] Int. Cl..... C22c 37/00

[58] Field of Search..... 75/123 K, 123 J

[56] **References Cited**

UNITED STATES PATENTS

1,261,742 4/1918 Churchward..... 75/123 K  
1,261,743 4/1918 Churchward..... 75/123 K  
2,026,418 12/1935 Crowe..... 75/123 K X  
2,060,765 11/1936 Welch..... 75/123 K X

2,150,785 3/1939 Rooke..... 75/123 K X  
2,707,680 5/1955 Succop..... 75/123 K

FOREIGN PATENTS OR APPLICATIONS

524,566 8/1940 Great Britain ..... 75/123 K

Primary Examiner—L. Dewayne Rutledge

Assistant Examiner—Joseph E. Legru

Attorney—F. Shapoe

[57]

**ABSTRACT**

An alloy is described which is suitable for use as a weld-filler material and which is characterized by having controlled strength and toughness. The composition includes about 4.5 percent nickel, 2 percent molybdenum, up to 0.35 percent carbon, low impurity and interstitial content, and the balance iron. The strength is controlled in accordance with the relationship:

0.2 percent yield strength = 52 K.s.i. + 268.4 K.s.i. C  
where C is the carbon content of a weldment made from the alloy in weight percent.

5 Claims, 2 Drawing Figures



PATENTED JAN 18 1972

3,635,698

SHEET 1 OF 2



Fig. 1

PATENTED JAN 18 1972

3,635,698

SHEET 2 OF 2



Fig. 2

WITNESSES

Helen M. Harkas

James T. Young

INVENTOR  
JULIUS HEUSCHKEL

BY Robert H. Bandy  
ATTORNEY



manganese, silicon, copper, chromium, vanadium, titanium, and cobalt, as well as low amounts of interstitial elements such as not more than about 0.004 percent phosphorus and sulfur, about 0.003 percent nitrogen and about 0.002 percent oxygen. The alloy in its welded condition is controlled so as to provide a 0.2 percent yield strength within the range between about 52 k.s.i. and about 200 k.s.i. in accordance with the relationship:

0.2 percent yield strength = 52 k.p.s.i. + 268.4 k.p.s.i.  $\sqrt{C}$   
where  $C$  is the carbon content in weight percent of the weld deposit.

#### DESCRIPTION OF THE DRAWING

FIG. 1 is a plot of the 0.2 percent yield strength and Charpy V-notch energy values versus the carbon content of the weld metal in the "as deposited condition"; and

FIG. 2 is a plot of the 0.2 percent yield strength and the Charpy V-notch energy versus the carbon content of the weldment after annealing for 8 hours at a temperature of 1,050° F. following welding.

#### DESCRIPTION OF THE PREFERRED EMBODIMENT

The alloy of the present invention is suitable for use as a weld-filler material and consists essentially of by weight from about 4.25 to about 4.75 percent nickel, from about 1.75 to about 2.25 percent molybdenum, up to about 0.35 percent carbon and the balance essentially iron. The alloy is characterized by having a 0.2 percent yield strength within the range between about 52 k.s.i. and about 200 k.s.i. in accordance with the relationship:

0.2 percent yield strength = 52 k.p.s.i. + 268.4 k.p.s.i.  $\sqrt{C}$   
where  $C$  is the carbon content in weight percent of the weld deposit. In this respect it should also be noted that it is necessary, and in fact highly critical, to maintain the interstitial content at as low a level as is practical commensurate with good metallurgical practice. In this respect, it is desired that the phosphorous and sulfur contents do not exceed about 0.04 percent, and the nitrogen content being less than about 0.003 percent and the oxygen content being less than about 0.002 percent. Typical levels of such other components include 0.05 max. silicon, 0.10 max. manganese, 0.05 max. copper, 0.3 max. chromium, 0.02 max. vanadium, 0.003 max. titanium, and 0.01 max. cobalt.

In order to more clearly demonstrate the alloy of the present invention, reference may be had to table I which lists a series of compositions of filler metals and weld deposits which were made and tested in accordance with the present invention.

In conducting these tests five experimental heats were

originally requested, the same to contain about 4.5 percent nominal nickel, 2.0 percent nominal molybdenum with a varying carbon content of 0.05, 0.10, 0.15, 0.20 and 0.25 weight percent carbon. All other elements were to be as near zero as possible, with the remainder of the alloy being iron. Actual chemical analysis indicates from table I that the nickel content ranged between about 4.25 and about 4.73 percent while the molybdenum content ranged between 2.08 and about 2.12 percent in the actual welding wires as the same were melted. However, insofar as the components of the weldment composition were determined, the nickel content ranged from 4.13 to about 4.67 percent while the molybdenum content varied between about 1.96 and about 2.23 percent. Thus it can be seen from the foregoing that a very good control can be maintained within the metal composition both in its steel-melting analysis as well as in the afterwelding weld metal analysis, the latter being in part influenced by the composition of the base metal being welded. The data contained in table I for the weld metal compared with the wire analysis indicates that excellent alloying component transference has occurred through the welding arc thereby assuring that the compositional quality of the weld can be accurately controlled.

The five experimental compositions were formed into welding wire and were converted into welds in an environment of pure argon using a tungsten arc to melt the wire to form the welds. These welds were utilized to join plates having the following composition:

|            |       |            |        |
|------------|-------|------------|--------|
| Carbon     | 0.17  | Nickel     | 3.53   |
| Manganese  | 0.35  | Chromium   | 1.64   |
| Phosphorus | 0.007 | Molybdenum | 0.29   |
| Sulfur     | 0.009 | Vanadium   | 0.11   |
| Silicon    | 0.23  | Nitrogen   | 0.0028 |
| Copper     | 0.11  | Oxygen     | 0.0018 |

35 The composition of each deposited weld as shown in table I is close to that of the corresponding wire, the primary difference being there was an increase in the copper and chromium content. This resulted from the fact that the plate contains a substantial amount of these two elements. With these relatively minor exceptions, the weld metals were essentially the same as the final composition of the corresponding weld wire used.

40 After welding, both tensile and impact specimens were made from these welds in both the as-deposited condition as well as after stress-relief-annealing of the weldment for about 8 hours at a temperature of 1,050° F.

45 Reference is directed to table II which lists the tensile and impact properties of the weldments employed in the "as-deposited" condition having the identification as set forth hereinbefore in table I.

TABLE II.—WELD METAL PROPERTIES (AS-DEPOSITED CONDITION)

| Loading cycle                            | Weld No.    |         |          |         |         |         |         |
|------------------------------------------|-------------|---------|----------|---------|---------|---------|---------|
|                                          | No. 1       | No. 1   | No. 1    | No. 2   | No. 2   | No. 1   | No. 1   |
| +80° F. tensile properties:              |             |         |          |         |         |         |         |
| Stresses (p.s.i.):                       |             |         |          |         |         |         |         |
| Prop. lim.                               | 126,000     | 142,200 | 174,000  | 198,750 | 194,500 | 200,000 | 190,000 |
| 0.2% yield                               | 131,100     | 160,400 | 190,800  | 202,000 | 202,500 | 207,000 | 200,000 |
| 0.5% yield                               | 130,800     | 173,400 | 197,000  | 197,000 | 198,000 | 206,500 | 200,250 |
| Ultimate                                 | 136,400     | 178,500 | 200,000  | 202,000 | 202,500 | 210,500 | 207,000 |
| True fracture                            | 321,500     | 337,800 | Unbroken | 335,800 | 350,850 | 334,300 | 313,700 |
| Ductility (percent):                     |             |         |          |         |         |         |         |
| Elong., YP                               | 1.75        | 4.18    |          |         |         |         |         |
| Elong., 2.5                              | 7.56        |         | 1.07     | 5.7     | 6.8     | 7.4     | 8.0     |
| Elong., unif.                            |             |         |          |         |         |         |         |
| Elong., total                            | 25.05       | 21.35   |          | 2 15.4  | 17.2    | 14.0    | 12.0    |
| Area red.                                | 79.10       | 68.80   | Unbroken | 59.2    | 60.2    | 54.4    | 44.8    |
| Charpy V-notch energy, values (ft.-lb.): |             |         |          |         |         |         |         |
| +200° F.                                 | 219.00      | 127.50  | 85.0     |         |         | 50.0    | 37.0    |
| +80                                      | 239.00      | 120.00  | 71.0     |         |         | 46.0    | 29.0    |
| +32                                      | 214.00      | 113.00  | 69.0     |         |         | 40.0    | 27.0    |
| 0                                        | 210.50      | 119.50  | 69.0     |         |         | 37.0    | 30.5    |
| -60                                      | 210.00      | 116.00  | 64.0     |         |         | 34.5    | 24.5    |
| -100                                     | 193.00      | 105.00  | 54.5     |         |         | 30.5    | 26.0    |
| -140                                     | 206 & 171.5 | 97.50   | 51.5     |         |         | 29.5    | 25.0    |
| -160                                     | 181.5       |         |          |         |         |         |         |
| -180                                     | 171.0       |         |          |         |         |         |         |
| -200                                     | 24 & 170.0  | 82.00   | 41.0     |         |         | 24.0    | 22.5    |

<sup>1</sup> Loading stopped at 200,000 p.s.i. and specimen transferred to larger testing machine designated as No. 2.

<sup>2</sup> True Total = 16.1%, i.e., 15.4 + 0.7%.

From the data set forth in Table II it becomes apparent that the alloy of the present invention has excellent strength together with excellent toughness even at temperatures below room temperature. In this respect it is noted that increasing the carbon content in the range indicated in Table I is effective for increasing the 0.2 percent yield strength from about 131 k.s.i. up to a value in excess of 200 k.s.i. This strength is attained with excellent elongation and reduction of area. Comitantly, it may be noted that with the higher carbon contents the toughness is reduced; however, it is noted that even at temperatures as low as -200° F. the metal still has in excess a 20 ft./lb. of energy absorbed, a condition which is highly desirable considering the demanding service condition arising at -200° F. temperature.

In order to more clearly demonstrate the outstanding strength and toughness properties exhibited by the alloy of the present invention, reference is directed to FIG. 1 which plots the carbon content of the weldment versus the yield strength and the Charpy V-notch energy absorbed both at room temperature and at a temperature of -60° F. In FIG. 1 the curve 10 represents the 0.2 percent yield strength while the curve 12 illustrates the Charpy V-notch energy curve when measured at a temperature of 80° F., and curve 14 is the same Charpy V-notch value when measured at a temperature of -60° F. From curve 10 it can be seen that the carbon content of the weldment has a well-defined relationship to the exhibited yield strength. Curve 10 indicates that the yield strength as measured will vary in the following manner:

0.2 percent yield strength = 52 k.p.s.i. + 268.4 k.p.s.i.  $\sqrt{C}$   
where  $C$  is the carbon content of the weldment in weight percent. This appears to be the equation which most closely predicts the yield strength based on the carbon content of the weld from the data contained in Table II and curve 10 in particular.

Thus, FIG. 1 indicates that an 80,000 p.s.i. yield-strength weld metal can be obtained using about 0.02 percent carbon in addition to about 4.5 percent nickel and 2.0 percent molybdenum. This provides a Charpy V-notch energy value of about 240 ft./lb. across the temperature range from -50° F. to +80° F. which constitutes an exceptionally high toughness level. Moreover, a 130,000 p.s.i. minimum yield-strength weld metal can be deposited by providing a minimum value of about 0.1 weight percent carbon. Such deposit results in a maximum impact energy value of 196 ft./lb. at -60° F. Similarly, a 150,000 p.s.i. minimum yield-strength weld deposit can be secured by the addition of a minimum of about 0.14 weight percent secured by the addition of a minimum of about 0.14 weight percent carbon, such carbon level resulting in an impact energy value of up to 145 ft./lb. at -60° F. Achievement of a level of about 20 ft./lb. at this last temperature is commonly considered to be in high strength weldments. In addition thereto, a

200,000 p.s.i. yield-strength weld deposit can be obtained with this alloy when a minimum of about 0.3 weight percent carbon is provided in the deposit. A weld deposit of such an alloy composition has an impact energy absorption of up to 38 ft./lb. at -60° F. Since in some cases, such as when residual welding stresses must be reduced to minimize or prevent stress corrosion cracking in a sea-water environment, it is desirable to thermally stress-relief-anneal a welded structure prior to use. This requires that the weld metal be able to withstand the imposed thermal cycling without excessive deterioration of its mechanical properties. An important criteria is not whether or not there is an actual loss or gain in the impact values as a consequence of the thermal treatment but rather, are the resulting values adequate to meet the intended service requirements. Ordinarily, a 50 ft./lb. value at +80° F. and a 20 ft./lb. value at -60° F. is considered adequate for very demanding service conditions.

Reference is now directed to Table 3 and FIG. 2, which illustrates the relationship between the carbon content and the yield strength as well as the Charpy V-notch energy absorption of the same materials after stress-relief-annealing for 8 hours at a temperature of 1,050° F. In FIG. 2 the curve 20 is a plot of the 0.2 percent yield strength versus the carbon content whereas the curve 22 is that of the Charpy V-notch energy versus the carbon content when measured at 80° F. and curve 24 is the same plot when measured at a temperature at -60° F. By comparing both curve 10 and curve 20 of FIGS. 1 and 2, respectively, it will be immediately apparent that the yield strength is directly related to the square root of the carbon content, the only difference being in the value of the zero carbon intercept between the material in the as-deposited condition and the material in the stress-relief-anneal condition. Thus, since the chemical composition can be controlled both in melting as well as in transference through the welding arc it becomes clear that a close control can be exercised over the quality of the welds made from materials produced in accordance with the teaching of the present invention.

Reference to FIG. 2 will indicate that such conditions are easily met by the composition of the present invention. Thus these data demonstrate that any desirable 0.2 percent yield strength within the 80 and 200,000 p.s.i. range can be obtained after a 1,050° F. soak for 8 hours with a slow heating and cooling cycle by the simple expedient of varying the carbon content to the proper level when the remainder of the weldment has the previously described composition. While the corresponding impact values are lower than those obtained for the as-deposited condition, these values are nevertheless above the minimum of 50 ft./lb. at 80° F. and 20 ft./lb. at -60° F. required for severe shock resistance conditions for 0.2 percent yield strength at levels of up to >190,000 p.s.i.

TABLE III.—WELD METAL PROPERTIES (ANNEALED 8 HRS. AT 1050° F.)

| Loading cycle                                                 | Weld No.      |               |                     |         |          |         |               |               |
|---------------------------------------------------------------|---------------|---------------|---------------------|---------|----------|---------|---------------|---------------|
|                                                               | 1374<br>No. 1 | 1375<br>No. 1 | 1375 R <sup>a</sup> |         | 1376     |         | 1377<br>No. 1 | 1378<br>No. 1 |
| 4-80° F. tensile properties:                                  |               |               |                     |         |          |         |               |               |
| Stresses (p.s.i.):                                            |               |               |                     |         |          |         |               |               |
| Prop. limit.....                                              | 124,400       | 153,400       | 162,000             | 180,300 | 167,800  | 177,900 | 195,000       | 215,450       |
| 0.2% yield.....                                               | 133,200       | 170,400       | 196,500             | 185,800 | 181,200  | 196,250 | 202,500       | 217,950       |
| 0.5% yield.....                                               | 134,800       |               |                     | 185,800 | 189,200  | 191,950 | 190,750       | 208,150       |
| Ultimate.....                                                 | 140,800       |               | 200,000             | 185,800 | 200,200  | 196,250 | 202,500       | 217,950       |
| True fracture.....                                            | 290,500       | 216,500       | Unbroken            | 289,000 | Unbroken | 277,150 | 242,150       | 263,650       |
| Ductility (percent):                                          |               |               |                     |         |          |         |               |               |
| Elongation:                                                   |               |               |                     |         |          |         |               |               |
| Uniform.....                                                  | 5.85          |               |                     | 0.43    |          | 0.2     | 0.1           | 0.1           |
| Total.....                                                    | 20.05         | 0.35          | 0.28                | 613.1   | 1.15     | 9.3     | 6.0           | 6.0           |
| Area reduction.....                                           | 72.20         | 19.16         | Unbroken            | 62.3    | Unbroken | 44.5    | 27.0          | 30.2          |
| Charpy V-notch energy (values ft. lb.) at temperature listed: |               |               |                     |         |          |         |               |               |
| +200° F.....                                                  | 110.0         | 65.0          |                     | 28.0    |          | 13.5    | 10.0          |               |
| +80° F.....                                                   | 105.5         | 65.0          |                     | 24.5    |          | 12.5    | 10.0          |               |
| +32° F.....                                                   | 114.0         | 56.0          |                     | 26.0    |          | 11.0    | 7.5           |               |
| 0° F.....                                                     | 107.0         | 65.5          |                     | 26.5    |          | 10.0    | 7.0           |               |
| -60° F.....                                                   | 110.5         | 63.0          |                     | 30.5    |          | 10.5    | 7.5           |               |
| -109° F.....                                                  | 122.5         | 55.0          |                     | 22.5    |          | 9.0     | 7.5           |               |
| -140° F.....                                                  | 26.0          | 43.0          |                     | 24.0    |          | 12.5    | 12.5          |               |
| -200° F.....                                                  | 25.0          | 44.0          |                     | 26.5    |          | 10.0    | 5.5           |               |

<sup>a</sup>1375 R is repeat test of 1375.

<sup>a</sup>Loading stopped at 200,000 p.s.i. and specimen transferred to larger testing machine designated as No. 2.

<sup>b</sup>True total-13.38%, i.e., 13.1-0.28%.

<sup>c</sup>True total-10.45%, i.e., 9.3-1.15%.

From the foregoing, it is clear that there has been provided a welding system wherein the alloy makeup and the balance itself to provide a built-in quality control with respect to properties, particularly above the 130 k.s.i. yield-strength level. Since the molybdenum and nickel contents are readily controllable both in the steel-melting practice and during transfer across the welding arc from the filler metal to the weld deposit, only variations in the carbon content significantly influence the final weld properties. Thus the alloy finds wide use in joining various ferrous base materials with only minor dilution which does not significantly affect the mechanical properties. Above about 0.10 percent carbon the strength response to carbon content variations is a minimum on a unit weight percent basis. By the simple expedient of making a check analysis percent basis carbon on each lot of welding wire, the probable weld deposit strength and toughness classification can be made thereby affording an excellent and accurately controlled prediction of weld quality.

In addition, the system is equally applicable for use in both the as-deposited or in the stress-relief-annealed conditions. The alloy system thus enables the attainment of controlled high-strength properties together with concomitant toughness properties in order to obtain an outstanding composition suitable for use as a weld-filler material.

I claim:

1. An alloy suitable for use as a weld metal consisting essentially of, by weight, from about 4.25 to about 4.75 percent nickel, from about 1.75 to about 2.25 percent molybdenum, up to about 0.35 percent carbon and the balance essentially iron, said alloy in the as-welded condition having a 0.2 percent yield strength within the range between about 52 k.s.i. and about 200 k.s.i. in accordance with the relationship:

0.2 yield strength =  $52 \text{ k.p.s.i.} + 268.4 \text{ k.p.s.i. } \sqrt{C}$   
 where  $C$  is the carbon content, in weight percent, of the weld deposit, said alloy being further characterized by low interstitial content and not exceeding about 0.004 percent phosphorus, about 0.004 percent sulfur, about 0.003 percent nitrogen and about 0.002 percent oxygen.

2. The alloy of claim 1 in which the nickel content is nominally about 4.5 percent and the molybdenum content is nominally about 2 percent.

3. The alloy of claim 1 in which the carbon content is limited to a range between about 0.10 percent and about 0.30 percent, said alloy having a minimum 0.2 percent yield strength of about 130 k.s.i. and Charpy V-notch impact energy value of about 40 ft.lb. at a temperature of  $-60^{\circ}\text{F}$ . in the as-deposited condition.

4. A weld rod suitable for producing high strength and high toughness in both the as-deposited and the stress-relief-toughness condition and formed of the alloy having the composition of claim 1.

5. A weld-filler material suitable for producing high strength and high toughness in a weldment, said material having a composition consisting essentially of, by weight, from about 4.25 to about 4.75 percent nickel, from about 1.75 to about 2.25 percent molybdenum, from about 0.10 to about 0.30 percent carbon and the balance essentially iron with not more than the following listed impurities:

|         |            |
|---------|------------|
| 0.004 % | phosphorus |
| 0.004 % | sulfur     |
| 0.003 % | nitrogen   |
| 0.002 % | oxygen     |

\* \* \* \* \*

35

40

45

50

55

60

65

70

75